

## UNITED STATES PATENT OFFICE

1,964,891

## PRODUCTION OF VISCOUS OILS

Mathias Pier, August Eisenhut, and Otto Eisenhut, Heidelberg, Germany, assignors to I. G. Farbenindustrie Aktiengesellschaft, Frankfort-on-the-Main, Germany, a corporation of Germany

No Drawing. Application September 6, 1928,  
Serial No. 304,382. In Germany September 28,  
1927

4 Claims. (Cl. 204—31)

This invention relates to the production of lubricating and insulating oils by treatment of oils, of any kind, which contain hydrocarbons, with high frequency electric currents.

5 A process has already been proposed for the production of viscous oils from substances of the nature of coal, tars, mineral oils and the like, in which the initial materials when solid are subjected to extraction or destructive hydrogenation, 10 and when liquid to destructive hydrogenation or cracking, and then subsequently to a high frequency treatment with or without the addition of catalysts.

We have now found that viscous products may 15 be obtained in a particularly advantageous manner from hydrocarbon oils from any source, by treatment in the liquid phase with high frequency electric currents, preferably high tension currents, when the treatment is carried out in the 20 presence of added finely divided solid carbonaceous materials such as powdered brown coal, powdered mineral coal, finely divided wood charcoal, colloidal or pulverulent metals, metal oxides, or coal ash or the like dispersed in the said oils 25 under treatment. The said additions apparently have a catalytic action, since the viscosity of the materials under treatment is increased in a much shorter time than without the said additions. Products of greatly improved quality are also 30 usually obtained by the said treatment. The above results are obtained even by the incorporation of very small amounts of said additions in the parent hydrocarbon oils. An addition of from one to five per cent of powdered coal will 35 usually suffice. In any event, amounts of the said additions which would render the oil under treatment conductive should not be employed.

The process may, for example, be carried out with an alternation number of 500 (=250 periods), but if desired, much higher frequencies, for example 2000 periods or more, may be employed with advantage.

The tension is adjusted according to the nature 45 of the product desired, and the kind of apparatus employed. For example the treatment may be carried out in a Voltol apparatus with a tension of about 2000 volts. When using ozonizing tubes 4000 volts or more, for example 10,000 or 12,000 50 volts may be employed.

The advantage of the present process consists in particular in an appreciable reduction in the time of reaction.

The following examples will further illustrate 55 how the invention may be carried into practical

effect but the invention is not restricted to these examples.

*Example 1*

A middle oil, prepared by destructive hydrogenation of crude oil from Elwerath, and of a boiling point range of 200°C. to 300°C., is subjected to a glow discharge of a tension of 2500 volts and of 2000 periods, in an atmosphere of an inert gas, for example of hydrogen in a Voltol apparatus and in the presence of about 2 per cent by weight of powdered brown coal as a suspension in the oil. The viscosity of the oil increases in a much shorter time of treatment than when operating under the same conditions but without the addition of brown coal. The economy in time amounts to 30 to 50 per cent. A valuable lubricating oil of suitable flashpoint and viscosity is obtained.

*Example 2*

A distillate, obtained from crude oil from Elwerath and having a boiling point between 185° and 250°C. and of quite low viscosity (1.1° Engler at 20°C.), to which about 2 per cent of powdered wood charcoal has been added is subjected to a high tension glow discharge in an ozonizing tube. A valuable product having a viscosity of 111° Engler at 20°C., 13° Engler at 50°C., 2.3° Engler at 100°C. and a suitable flashpoint and tar number is obtained from the mixture thus treated by 85 centrifuging or filtering off the powdered wood charcoal.

What we claim is:

1. Process for converting hydrocarbon oils into lubricating and insulating oils which comprises subjecting said oils, in the liquid state and in the presence of substantial quantities of added finely divided substances selected from the group consisting of finely divided solid carbonaceous materials, colloidal and pulverulent metals and metal oxides dispersed in the oils under treatment, to the action of a glow discharge the quantity of the added finely divided substances being such that the oils under treatment do not become electrically conductive.

2. Process for converting hydrocarbon oils into lubricating and insulating oils which comprises subjecting said oils, in the liquid state and in the presence of about 1 to 5% of finely divided substances selected from the group consisting of finely divided solid carbonaceous materials, colloidal and pulverulent metals and metal oxides dispersed in the oils under treatment, to the action of a glow discharge.

3. Process for converting hydrocarbon oils to

lubricating and insulating oils which comprises subjecting said oils, in the liquid state and in the presence of about 1 to 5% of finely divided brown coal dispersed in said oils, to the action of a glow discharge.

4. Process for converting a middle oil obtained by the destructive hydrogenation of crude oil and having a boiling point range of 200 to 300°C. into lubricating and insulating oils which comprises

10

subjecting said middle oil to a glow discharge in an atmosphere of hydrogen and in the presence of from 1 to 5% of finely powdered brown coal suspended in said oil, said discharge being induced by a current of 2500 volts and a frequency of 2000 periods.

80

MATHIAS PIER.  
AUGUST EISENHUT.  
OTTO EISENHUT.

85

15

90

20

95

25

100

30

105

35

110

40

115

45

120

50

125

55

130

60

135

65

140

70

145

75

150